

M. M. MERRITT.  
ELECTROLYTIC PROCESS AND PRODUCT.  
APPLICATION FILED DEC. 8, 1917.  
1,282,268. Patented Oct. 22, 1918.

*Fig. 1.*



*Fig. 2.*



INVENTOR:  
Matthew M. Merritt.  
by Emery Booth Janney & Verney  
Attys.

# UNITED STATES PATENT OFFICE.

MATTHEW M. MERRITT, OF SOUTH MIDDLETON, MASSACHUSETTS, ASSIGNOR TO COPPER PRODUCTS COMPANY, OF BOSTON, MASSACHUSETTS, A CORPORATION OF MAINE.

## ELECTROLYTIC PROCESS AND PRODUCT.

1,282,268.

Specification of Letters Patent. Patented Oct. 22, 1918.

Original application filed November 2, 1917, Serial No. 199,808. Divided and this application filed December 8, 1917. Serial No. 206,292.

To all whom it may concern:

Be it known that I, MATTHEW M. MERRITT, a citizen of the United States, and a resident of South Middleton, county of Essex, Commonwealth of Massachusetts, have invented an Improvement in Electrolytic Processes and Products "A," of which the following description, in connection with the accompanying drawings, is a specification, like characters on the drawings representing like parts.

This invention pertains to improvements in electrolytic processes and products, and more particularly, though not exclusively, to improvements in the art of electrolytically depositing copper or other metal on the surfaces of non-conductive bodies such as bodies composed of wood.

The invention is peculiarly useful as applied to electrolytically coating with copper the surface of aeroplane propellers.

This application is a divisional of my co-pending application, Serial No. 199,808, filed Nov. 2, 1917.

25 In the drawings that show one form of an illustrative embodiment of my invention:

Figure 1 shows an aeroplane propeller coated with copper; and

30 Fig. 2 is a diagrammatic section therethrough on the line 2-2 of Fig. 1.

I have found that when an aeroplane propeller is coated with an electrically conductive coating such as precipitated bronze 35 powder and amyl-acetate, or any of the more usual substitutes therefor, and electrolytic deposits of copper are made thereon, that the structure of the deposited copper is relatively coarse, and the sheet of

40 copper comparatively brittle. I believe this to be due to the comparatively coarse structure of the bronze powder, there being a tendency for the deposited copper to partake of the general structure, so far as 45 coarseness is concerned, of the electrically conductive body on which it is deposited. The life of the copper coating on an aeroplane propeller depends on its toughness and fineness of structure. I have found

50 that a very tough coating of electrolytically deposited copper may be deposited by initially depositing on the electrically conductive paint or the like, a layer of copper,

preferably comparatively thin, amalgamating this copper surface with mercury or 55 with a mercury amalgam, and then depositing on the amalgam surface a second layer or lamination of copper.

The second layer of copper is of very fine-grained, close texture because the initially 60 coarse first copper coating has been rendered fine-grained by the application of the mercury or mercury amalgam.

It is incontrovertible that the application of mercury or mercury amalgam to a copper 65 sheet renders the copper sheet brittle and greatly reduces its tensile strength. This weakening of the copper structure is probably due to the penetration of the mercury between the pores of the copper with resultant reduction of the cohesion of the copper. In making the experiments leading up to the present invention, I had expected that the first sheet of copper would be so weakened by the mercury that it would contribute 70 practically no strength to the structure. I found, however, on stripping a blade made in accordance with the present invention, that the deleterious effect of the mercury on the initial copper coating appears to be corrected or, in any case, greatly reduced by the combined action of the electrolyte and the current during the subsequent electro-deposition, leaving the initial coating of copper 75 very ductile and strong. The effect of the mercury between the first and second coating is to laminate the structure and I may, if desired, continue the laminations by amalgamating the surface of the deposited metal 80 several times, thus producing a copper reinforcement for the propeller having any 85 desired number of laminations.

In my co-pending application, filed herewith, I have described the use of grease in various ways to produce fineness of texture 95 of the successive copper deposits and, if desired, to effect laminations therein. It will be understood that the present invention, and that described in my co-pending application, may be used in conjunction with one 100 another or alternatively, the generic dominating claims being included in this application.

While I have shown and described one embodiment of my invention, it will be understood that I may greatly vary the same with-

out departing from the scope of my invention, which is best defined in the following claims:—

Claims:

5. 1. The method of electrolytically coating non-conductive cathodes which comprises applying to the surface thereof an electrically conductive substance, electrolytically depositing a layer of metal thereon, applying a foreign substance of relatively low tensile strength to the surface of said initial layer of electrolytically deposited metal and continuing electro-deposition to provide a second laminated layer of deposited metal 15 separated from the first by said foreign substance.
10. 2. The method of electrolytically coating non-conductive cathodes which comprises applying to the surface thereof an electrically conductive substance, electrolytically depositing a layer of metal thereon, amalgamating with mercury the surface of said deposited layer, and electro-depositing a second coating of metal on the amalgamated 20 surface.
15. 3. The method of electrolytically coating non-conductive cathodes which comprises
25. applying to the surface of the cathodes an electrically conductive paint, electro-depositing a comparatively coarse-grained layer of copper on said paint, amalgamating with mercury the surface of said relatively coarse-grained layer of copper, and subsequently depositing a second layer of copper, whereby said second layer of copper partaking of the fine texture of the amalgamated surface may be of fine grain and of relatively greater strength than the initial layer of copper.
30. 4. The method of electrolytically coating flexible cathodes, which comprises depositing thereon successive layers of metal separated by foreign substances of relatively low tensile strength, whereby successive laminations of metallic layers are provided.
35. 5. The method of toughening electrolytic deposits, which comprises coating said deposits with mercury and passing an electric current therethrough, while subjected to the action of an electrolyte.

In testimony whereof I have signed my name to this specification.

MATTHEW M. MERRITT.